

## UNITED STATES PATENT OFFICE

2,270,192

## MAGNESIUM BASE ALLOY

John C. McDonald, Midland, Mich., assignor to  
The Dow Chemical Company, Midland, Mich.,  
a corporation of Michigan

No Drawing. Application December 23, 1940,  
Serial No. 371,374

4 Claims. (Cl. 75—168)

The invention relates to magnesium base alloys and more particularly concerns an alloy of this nature having highly improved tensile and yield strengths associated with a sufficient degree of formability or ductility to permit its being subjected to forming operations.

Magnesium base alloys are being widely used in the structural arts where a light weight metal is highly desirable, such as for use in making castings, forgings, and the like. However, the use of these alloys in the rolled form to make sheet metal articles requiring forming operations, such as bending and drawing, has not progressed as rapidly due to the fact that, in general, alloys having good formability or ductility permitting relatively sharp bends to be made without the article developing external cracks usually have inferior characteristics as regards their tensile and yield strengths.

It is, accordingly, the principal object of the invention to provide a magnesium base alloy which can be made into rolled sheets and the like possessing a sufficient degree of ductility or formability at ordinary temperatures to be

strengths coupled with satisfactory formability are manifest over the entire range of composition indicated, I have found that in general an alloy containing from about 0.05 to 0.5 per cent of calcium, 1.5 to 2.5 per cent of manganese, and from 3 to 8 per cent of thallium, possesses the most satisfactory combination of properties. A particularly desirable composition is one containing 0.15 per cent of calcium, 2 per cent of manganese, and 5 per cent of thallium.

The following table listing some of the properties of rolled sheet metal made from my new quaternary alloy and comparing these properties with those of related ternary alloys, illustrates the improvement in strength characteristics of my new alloy over that of related commercial alloys and at the same time shows that the per cent elongation, which is to be regarded as a measure of the formability, is of a sufficiently high order to permit the article to be subjected to forming operations.

In the following table the per cent elongation is to be regarded as a measure of the formability or ductility of the alloys.

Table

| Nominal composition in percent (remainder=magnesium) |     |     | Annealed                       |                                |                                  | Cold rolled                    |                                  |
|------------------------------------------------------|-----|-----|--------------------------------|--------------------------------|----------------------------------|--------------------------------|----------------------------------|
| Ca                                                   | Mn  | Tl  | Percent elongation in 2 inches | Yield strength in lbs./sq. in. | Tensile strength in lbs./sq. in. | Yield strength in lbs./sq. in. | Tensile strength in lbs./sq. in. |
| ---                                                  | 2.1 | 5.2 | 10                             | 22,000                         | 38,000                           | 31,000                         | 39,000                           |
| 0.15                                                 | 5.0 | 15  | 21,000                         | 35,000                         | 31,000                           | 35,000                         |                                  |
| 0.11                                                 | 2.2 | 5.0 | 14                             | 25,000                         | 38,000                           | 34,000                         | 41,000                           |

sharply bent, drawn, or otherwise shaped, while having highly improved tensile and yield strengths.

Other objects and advantages will be apparent as the description of this invention proceeds.

My invention resides in the discovery that a magnesium base alloy containing from 0.01 to 1 per cent of calcium, 0.01 to 3 per cent of manganese, and from 1 to 12 per cent of thallium possesses the aforementioned desirable properties. The term "magnesium" used herein and in the appended claims is intended to include magnesium containing the ordinary impurities found in the commercially pure metal, such as traces of copper, silicon, nickel, and iron.

While the properties of high tensile and yield

strengths coupled with satisfactory formability are manifest over the entire range of composition indicated, I have found that in general an alloy containing from about 0.05 to 0.5 per cent of calcium, 1.5 to 2.5 per cent of manganese, and from 3 to 8 per cent of thallium, possesses the most satisfactory combination of properties. A particularly desirable composition is one containing 0.15 per cent of calcium, 2 per cent of manganese, and 5 per cent of thallium.

The properties set forth above under the term "annealed" were obtained by first rolling specimens of the alloys at a temperature of 550° F. and thereafter annealing them at various temperatures in a range of from 400° to 300° F. The properties selected for the table were those of the annealed specimens which exhibited the maximum elongation. The properties set forth under the term "cold rolled" were obtained by subjecting specimens of the alloys which had first been hot rolled at temperatures of 550° F. to additional rolling in the cold state. The properties selected for the table were those of the cold rolled specimens which exhibited the greatest tensile and yield strengths, while having at least 1 per cent elongation in 2 inches.

A comparison of the properties listed in the table shows that the yield and tensile strengths in both the annealed and cold rolled state is markedly superior to those of related alloys, while it will be noted that the per cent elongation is only slightly inferior to that of the related alloys showing the highest degree of formability.

The new alloy may be compounded by any of the methods usually employed for melting and alloying metal with magnesium, such as by adding the alloying ingredients singly or jointly to a bath of molten magnesium which is preferably protected from oxidation by a suitable flux. The flux should be substantially free from magnesium chloride if the calcium content of the alloy is above 0.3 per cent. In those instances where the alloy is to be compounded containing less than 0.3 per cent of calcium, magnesium chloride may be present in the flux, but in this case it is preferable to add the calcium last and without too much stirring and agitation to prevent loss of calcium into the flux.

It is to be understood that the invention is not limited to the specific composition herein

described but may take other forms without departing from the scope of the invention.

I claim:

1. A magnesium base alloy containing from about 0.01 to 1 per cent of calcium, from about 0.01 to 3 per cent of manganese, and from 1 to 12 per cent of thallium, the balance being magnesium.
2. A magnesium base alloy containing from about 0.05 to 0.5 per cent of calcium, from 0.5 to 2.5 per cent of manganese, from 3 to 8 per cent of thallium, the balance being magnesium.
3. A magnesium base alloy containing 0.15 per cent of calcium, 2 per cent of manganese, 15 5 per cent of thallium, the balance being magnesium.
4. A magnesium base alloy containing from 0.01 to 1 per cent of calcium, about 0.01 to 3 per cent of manganese, and about 1 to 12 per cent of thallium and characterized by improved tensile strength and yield strength as compared to a similar magnesium-calcium-manganese alloy devoid of thallium.

JOHN C. McDONALD.